

March 18, 1969

M. J. D'ERRICO ET AL 3,433,658  
WARM WATER-DILUTABLE PASTE ROSIN SIZE AND PROCESS  
FOR THE MANUFACTURE THEREOF  
Filed Jan. 17, 1968



INVENTORS.  
MICHAEL J. D'ERRICO  
RUSSELL J. KULICK  
BY

*Evanekahn*

ATTORNEY

3,433,658

**WARM WATER-DILUTABLE PASTE ROSIN SIZE AND PROCESS FOR THE MANUFACTURE THEREOF**

Michael Joseph D'Errico, Stamford, Conn., and Russell Joseph Kulick, Lee, Mass., assignors to American Cyanamid Company, Stamford, Conn., a corporation of Maine  
Continuation-in-part of applications Ser. No. 413,603, Nov. 24, 1964, and Ser. No. 584,194, Oct. 4, 1966.  
This application Jan. 17, 1968, Ser. No. 698,655  
U.S. Cl. 106—123 8 Claims  
Int. Cl. D21c 3/00; C11d 15/04; C09f 1/04

**ABSTRACT OF THE DISCLOSURE**

A fluid rosin size consisting of an aqueous dispersion of a rosin saponified at least 85% with an alkali metal of which at least about 75 mol percent of the metal cations are potassium, and 9–20% of an anti-gel agent selected from the group consisting of ethanol and iso-propanol, the rosin size solids content of said size being between about 65% and 80% by weight.

This is a continuation-in-part of our copending applications Ser. Nos. 413,603 and 584,194, respectively filed on Nov. 24, 1964 and Oct. 4, 1966 and now abandoned.

The present invention relates to paste rosin size of improved fluidity and of improved dilutability with water to a solids content of less than 10% by weight. More particularly, the present invention relates to paste rosin size which is of pumpable viscosity at normal storage temperature and which in preferred instances is of pumpable viscosity at room temperature, and which can be readily diluted with warm and in preferred instances with cold water to a solids content of less than 10% by weight, and to processes for manufacturing and diluting such size.

Rosin size is customarily manufactured by partially neutralizing a papermaker's rosin (gum rosin, tall oil rosin, fumarated rosin, formaldehyde-reacted rosin, etc.) with aqueous sodium hydroxide solution. The amount of sodium hydroxide is predetermined so that the rosin is neutralized or "saponified" to the extent of about 75%–85% and the amount of water is predetermined so that the resulting size is barely of pumpable viscosity at normal storage temperature (170° F. or 71° C.) to avoid the necessity of shipping more water than is absolutely necessary. The resulting rosin is termed "paste" rosin size, and contains about 65%–80% rosin size solids by weight. Check U.S. Patent No. 3,321,325. It is a sticky almost solid mass at room temperature, but becomes a viscous pumpable fluid when hot. It is consequently prepared for shipment at as high a temperature as is practical (in the range of 150° F.–210° F.) and is shipped sufficiently rapidly so that it is of pumpable viscosity when received by the user.

Paste rosin size is generally transported by tank cars and is discharged from the cars by pumping. The cars are thermally insulated but receive no heat. They consequently cool in transit more or less, depending on the length of the trip and the season of the year. If the size arrives at a non-pumpable viscosity when received by the user, it must be re-heated, and this is a slow and inconvenient task, which, if not performed carefully, may "burn" the size.

Moreover, the size must be diluted to low (2%–5%) solids content before it can be used in papermaking. Dilution of paste rosin size with cold water presents a serious difficulty, which arises as follows.

When a quantity of hot paste rosin size is mixed with a quantity of cold water, the size transforms itself into a stiff gel, after which further dilution of the size becomes difficult and slow. This phenomenon is generally regarded as independent of the extent to which the rosin has been saponified and occurs even in the case of a rosin size wherein the rosin is completely saponified, so that the rosin size contains no free rosin acids at all. The phenomenon is described more in detail in Howell U.S. Patent No. 2,573,024 (1951), which discloses a number of expedients for overcoming this difficulty.

The discovery has now been made that rosin size which consists essentially of an aqueous dispersion of a rosin which is at least 85% saponified with an alkali metal alkali at least about 75 mol percent of the metal cations of which are potassium, and which contains between about 2% and 20% (based on the weight of rosin size solids in the size) of a water-soluble saturated monool, is fluid (i.e., is of pumpable viscosity) at standard storage temperatures when of rosin size solids content between 65% and 85% by weight, yet is readily dilutable with warm (40° C.) water and in preferred instances with cold and even with ice water through the range of solids at which formation of a stiff slow-dissolving gel would otherwise occur. In other words, we have discovered that paste rosin size of the composition described does not pass through a viscous gel stage when it is extensively diluted with water in any amount.

The size of the present invention possesses the following advantageous properties:

(1) It can be diluted to as low as 1%–5% solids by introducing the size, at a temperature at which it is fluid, into an appropriate amount of warm water or in preferred instances cold water with gentle agitation (e.g., sufficient agitation to break up the size into small globules). The globules dissolve within a few minutes; the result is a clear soap solution. As a result, an excellent size solution is easily and quickly obtained at high dilution direct from paste rosin size without need for special equipment.

(2) The invention permits a major economy in the handling of rosin size. Heretofore, tank cars of rosin size have typically required 36 hours to be discharged at 160° F. The size of the present invention, because of its greater fluidity, can be discharged under similar conditions in 6 hours. Moreover, in preferred instances, sizes of the present invention at solids content of 70% or more are of pumpable viscosity at temperatures down to 60° F. Hence tank cars containing such size can usually be discharged at the temperatures at which they are received by the customer, and need not be reheated.

(3) The size of the present invention is used in the manufacture of paper in the same manner as ordinary rosin size, and the paper manufacturer need not learn any new techniques. Paper having a content of the size of the present invention is of normal appearance and properties.

The invention is further illustrated by the drawing, which is a three-dimensional graph showing the principal parameters of rosin size in general (parameters A, B, and C), of the size of the present invention viewed generically (parameters D, E, and F), and of one preferred embodiment of rosin size of the present invention (parameters G, H, and I).

In the drawing, parameter A represents the mol percent of potassium ions which may be present in rosin size (based on the total number of mols of metal ions present); parameter B represents the weight of saturated monool which may be present based on the weight of rosin size solids in the size, and parameter C represents the extent (mol percent) to which the rosin in the size has been saponified.

Parameters D, E, F define the rosin size of the present invention generically. As shown by parameter D, at least about 75 mol percent of the metal ions in the size are potassium ions. As shown by parameter E, the size contains between about 2% and 20% of a saturated monoool based on the weight of the size solids in the size. As shown by parameter F, the rosins in the size are at least about 85% saponified. The sizes thus defined are of pumpable viscosity at normal storage temperatures and rapidly and completely dissolve to 1% solids when gently stirred in water at 40° C.

In one preferred size illustrated, at least 85 mol percent of the metal ions are potassium ions as is shown by parameter G, the amount of the monoool is 9% to 12% of the weight of rosin size solids in the size as is shown by parameter H, and the amount of the rosin which is saponified is at least 85%. This size at rosin size solids content of 60%-75% is fluid at room temperature and dissolves to 1% solids readily even in water at room temperature. It may but need not contain a larger proportion of monoool.

In another instance, the size is of about 80% rosin solids size content, the rosin therein is 85%-90% saponified. The weight of the monoool is 2%-4% of the weight of rosin size solids in the size, and more than 95 mol percent of the metal ions in the size are potassium ions. Such size, although containing a very small amount of monoool, dissolves readily to 1% solids in warm (50° C.) water.

When the rosin is more than 95% neutralized, when more than 95 mol percent of the metal ions are potassium, and when the amount of monoool is 9%-20% of the weight of size solids, the size is of pumpable viscosity at room temperature and is readily soluble in ice water.

When the proportion of potassium cations to all the metal cations present in any given size of the present invention is decreased below about 75%, the size becomes unduly difficult to disperse even in warm water, and hence the resulting size is outside the present invention.

When the amount of saturated monoool and the extent of saponification of the rosin are below the indicated minimum in any instance, the size tends to form a stiff gel on admixture with water, and such size too is outside the present invention. Excess monoool (i.e., more than 20% based on the weight of size solids) is disadvantageous because the excess monoool increases the unit cost of the size without contributing any significant off-setting advantage. On the other hand the rosin may advantageously be substantially completely saponified, and substantially complete saponification is preferred where lowest fluidity and maximum ease of dispersibility in water are desired.

The term "cation" as used in the present application designates not merely metal ions in dissociated state, but also metal in combined rosinate form as, for example, in potassium rosinate. Preferably, substantially all the cations of the size of the present invention are potassium as in such instance the size possesses better dispersibility than would otherwise be the case.

The saturated monoools which are present in the size of the present invention include the water-soluble C<sub>1</sub>-C<sub>4</sub> alkanols, for instance methanol, ethanol, propanol, isopropanol, butanol, t-butanol, and isobutanol, and saturated lower monohydric alcohols such as 3-chloro-1-propanol, 2-methoxyethanol, ethanolamine, and 2-nitroethanol. Mixtures of these or other similar lower monoools may be used. So far, isopropyl alcohol has proved the most effective monoool on a cost basis and possesses nearly the effectiveness of ethanol without possessing its great volatility and is therefore preferred. Humectant diols (for example, ethylene glycol and glycerol) predispose the rosin sizes of the present invention to gel when diluted with water, and therefore should not be used.

The monoool content of the size is at least that amount which prevents formation of a viscous gel when the size is diluted with water. For this purpose, 2% of the monoool is about the least amount which is effective. Size containing

this amount of monoool is of pumpable viscosity and the gel which it forms when it is mixed with water dissolves rapidly. On the other hand it is generally unnecessary for the amount of monoool to be more than about 12% of the weight of the rosin size solids, and the latter amount is therefore regarded as satisfactory to most commercial users.

We have found that sizes containing 9%-12% of the monoool and substantially no free rosin acid are especially beneficial when the only metal cation present is potassium. In such event, the size possesses the most important and surprising properties of being a mobile liquid at room temperature and at 70% solids, and of dispersing rapidly in ice water with no more than moderate agitation. The amount of monoool may advantageously be larger, up to about 20%, and such larger amount is specially advantageous when the size is to be pumped long distances in cold weather.

The paste rosin size of the present invention can be manufactured by saponifying any of the numerous paper-maker's rosins (such as have been named above) with an alkali at least 75% of the cations of which are potassium, and adding a saturated monoool, the amounts of water, monoool and alkali, and the proportion of potassium cations to the other metal ions therein, being predetermined so that the size falls within the parameters D, E, and F of the drawing and is of pumpable viscosity at 170° F. while having a rosin size solids content of at least 60% by weight.

Suitable proportions are readily established in any instance by preparing a series of sizes in the laboratory, and determining the viscosity of the size and the amount and solubility of the gel which it forms during dilution with water. Formation of insoluble or slow-dissolving gel or too high a viscosity indicates that the composition should be modified in the direction of parameters G, H and I.

In rosin size manufacture, the term "pumpable viscosity" is generally taken to mean a viscosity of about 3,500 centipoises (Hoeppler), but in special instances a size of higher viscosity is regarded as pumpable, depending on the power of the pump which is available, the length of pipe through which the size must be pumped, the number of bends in the pipe, etc.

The saturated monoools generally do not react with the alkali or with the rosin or rosin size. Consequently they can be introduced during or after saponification. However, they are volatile at the temperatures at which rosin is saponified, and hence in instances where the saponification step is performed in an open vessel, they are most conveniently metered into the size as it is pumped into closed storage tanks or into tank cars for shipment.

When the size is made in a continuous saponifier such as is shown in Anderson et al. U.S. Patent No. 2,842,453 the alkanol may be introduced as a component of the caustic solution or into the discharge from the saponifier as preferred.

Dilution of the rosin size of the present invention is readily affected in one step from 60%-80% rosin size solids by weights to 2%-5% rosin size solids by agitating the size with an appropriate quantity of water. The temperature of the water should be that at which the size undergoes rapid and complete dispersion. Homogenization or even intensive agitation is not required. If preferred, a continuous stream of dilute size can be provided by introducing the size as a fine stream into water in turbulent flow. The minimum suitable temperature of the water in any instance can be determined by introducing the size through a hypodermic needle into a beaker of water agitated by a propeller-type stirrer operating at moderate speed. Formation of globules of size which dissolve rapidly and completely show that the water is of suitable temperature. Slow or partial dissolution of the size shows that the temperature of the water should be raised.

The monool does not appear in the paper when the size is employed in papermaking, but remains in the white water. The monool thus has no significant effect upon the amount of water resistance, lactic acid resistance, etc., which is imparted by the size.

The paste rosin size of the present invention may contain minor amounts of other materials such as are customarily present in paste rosin size, for example, sodium

side wall of the beaker to act as baffle. Sizes are regarded as dispersible when a clear solution or dispersion forms within three minutes. The presence of floc or other insoluble matter in the water at the end of three minutes is evidence of only partial dissolution of the size and indicates that the size is unsatisfactory.

The tests show that the sizes can be satisfactorily dispersed in water without homogenization.

| Run No. | Rosin                                                         | Description of Sizes <sup>1</sup> |                                             |                      | Percent<br>K <sup>3</sup> | Saturated Monool | Autodilutability <sup>4</sup> in H <sub>2</sub> O |        | Appearance<br>of Solutions |
|---------|---------------------------------------------------------------|-----------------------------------|---------------------------------------------|----------------------|---------------------------|------------------|---------------------------------------------------|--------|----------------------------|
|         |                                                               | Percent<br>Solids                 | Percent<br>Rosin<br>Saponified <sup>2</sup> | Percent <sup>4</sup> |                           |                  | 20° C.                                            | 50° C. |                            |
|         | Tall oil <sup>6</sup>                                         | 75                                | 90                                          | None                 |                           |                  | N.G.                                              | N.G.   | ( <sup>7</sup> ).          |
|         | Gum                                                           | 75                                | 90                                          | 100                  |                           |                  | N.G.                                              | N.G.   | ( <sup>7</sup> ).          |
| 1       | Gum                                                           | 75                                | 90                                          | 100                  | 1                         | Isopr OH         | N.G.                                              | N.G.   | ( <sup>7</sup> ).          |
| 2       | Gum                                                           | 75                                | 90                                          | 100                  | 2                         | do               | N.G.                                              | O.K.   | Clear.                     |
| 3       | Gum                                                           | 75                                | 90                                          | 100                  | 3                         | Et OH            | N.G.                                              | O.K.   | Do.                        |
| 4       | Gum, fumarated <sup>7</sup>                                   | 75                                | 90                                          | 100                  | 3                         | Pr OH            | N.G.                                              | O.K.   | Do.                        |
| 5       | do                                                            | 75                                | 90                                          | 100                  | 2                         | Isopr OH         | N.G.                                              | O.K.   | Do.                        |
| 6       | do                                                            | 75                                | 95                                          | 75                   | 2                         | do               | N.G.                                              | O.K.   | Do.                        |
| 7       | do                                                            | 75                                | 85                                          | 100                  | 4                         | do               | O.K.                                              | O.K.   | Do.                        |
| 8       | Tall oil, CH <sub>2</sub> O and isom. <sup>8</sup> reacted in | 75                                | 90                                          | 100                  | 2                         | do               | N.G.                                              | O.K.   | Do.                        |
| 9       | do                                                            | 75                                | 85                                          | 100                  | 4                         | do               | O.K.                                              | O.K.   | Do.                        |
| 10      | do                                                            | 75                                | 100                                         | 100                  | 5                         | do               | O.K.                                              | O.K.   | Do.                        |
| 11      | Tall oil, fumarated <sup>7</sup>                              | 75                                | 90                                          | 100                  | 3                         | do               | N.G.                                              | O.K.   | Do.                        |
| 12      | do                                                            | 75                                | 95                                          | 100                  | 4                         | do               | O.K.                                              | O.K.   | Do.                        |

<sup>1</sup> Based on the weight of the size.

<sup>2</sup> Mol percent of rosin acids saponified.

<sup>3</sup> Metal cation content (mol percent) of size.

<sup>4</sup> Based on weight of solids in size.

<sup>5</sup> For description of test, see text above.

<sup>6</sup> Tall oil rosin isomerized at 275° C. for 30 minutes.

<sup>7</sup> Tall oil rosin reacted with  $\frac{1}{2}$  mol of fumaric acid at 200° C.

<sup>8</sup> Tall oil rosin reacted with  $\frac{1}{2}$  mol of paraformaldehyde at 150° C. and heated for 30 minutes at 275° C.

<sup>9</sup> Size does not dissolve. When stirring stops, size droplets settle to bottom of beaker and form a layer.

or potassium acetate, chloride or nitrate, as fluidifying assistants; pentachlorophenol as mold growth inhibitor, a cationic resin or limonene as auxiliary fortifier; and emulsified wax or a hydrophobic synthetic thermoplastic resin as a supplementary size.

The invention will be further illustrated by the examples that follow. These examples are illustrations of the invention and are not to be construed as limitations thereon.

#### Example 1

The following illustrates a number of rosin sizes according to the present invention which are fluid at 170° F. and which dissolve completely 1% solids without homogenization rapidly in warm or cold water in one step, 45 without formation of slow-dissolving gel.

The sizes are prepared by saponifying a rosin with aqueous potassium hydroxide (or with an aqueous mixture of potassium hydroxide and sodium hydroxide); the amounts of alkali and water are pre-determined so that the free acid content and size solids content in the resulting size is as shown in the table below, which also shows the particular rosin which is saponified in each instance and the mol percent of potassium ions in the size. There is then stirred into the sizes at 70° C. a C<sub>2</sub> or C<sub>3</sub> 55 saturated monool, as is shown in the table below.

Control sizes are prepared without use of potassium alkali or any saturated monool, and a control size is prepared by use of a potassium alkali but with an insufficient amount of monool.

The control sizes do not dissolve in water at 50° C.

The remaining sizes which exemplify sizes of the present invention dissolve readily when 10 parts (or less than 10 parts) by weight of the sizes are stirred into 90 parts of water at 50° C. In several instances (where the rosin is more than 90% saponified and the amount of alkanol present is 8-12% of the weight of size solids), the sizes dissolve readily when the temperature of the water is 25° C. or less.

The dispersibility test is performed by dropping 1.0 g. 70 of size at 65° C. from a hypodermic syringe into 99 g. of water having the temperature shown in the table contained in a 250-cc. laboratory beaker rotating from the effect of a magnetic capsule turning at 1500 r.p.m. and then placing a 1/2" wide spatula vertically along the in-

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

open vessel by adding thereto a solution of 70 g. of potassium hydroxide in 130 g. of water. A fluid rosin size of 75% solids and 8% free rosin acid content is obtained. There is then added with stirring 15.0 g. (4% on the weight of sizing solids) of isopropyl alcohol. The viscosity of the product is such that it is a fluid viscosity at 20° C.

The size dissolves rapidly when aspirated through a pipe  $\frac{1}{16}$ " in diameter into water at 20° C. flowing at a brisk pace from a laboratory faucet through a pipe about  $\frac{1}{4}$ " in inside diameter. The discharge from the pipe is a clear solution and contains about 7% by weight of rosin size solids.

#### Example 4

The following illustrates the preparation of a preferred size of the present invention and the outstanding solubility properties which it possesses.

To 100 g. of tall oil rosin at 200° C. is added 16 g. of fumaric acid with stirring, and the mixture is maintained at 200° C. for 2 hours. To the product is added 300 g. of tall oil rosin which had previously been reacted with 2% by weight of paraformaldehyde at 160° C. and then heated at 275° C. for 30 minutes.

The resulting mixture is cooled to 125° C. and is substantially 100% saponified by addition of 78.4 g. of potassium hydroxide in water.

To the resulting size is added 11.6 g. of potassium chloride, 48 g. of isopropyl alcohol (10% on the weight of size solids) and sufficient water to adjust the solids content of the size to 70%.

The resulting size has a viscosity of less than 200 centipoises at 71° C. and is of pumpable viscosity (ap-

Six aliquots each weighing 89.8 g. (and containing 67.6 g. of size solids) are removed. To each is added with stirring 6.8 g. of one of the monoools shown below. The samples each contain 10% of monool based on the dry weight of the solids therein; the products are paste rosin size containing 70% solids by weight. The samples are placed in 100 cc. vials which are capped and cooled to 25° C.

The presence or absence of gel in the samples of size is determined in each instance by observing the flow made of the size when a cylindrical vial is quarter-filled with a sample of the size at 18° C. and the vial is up-ended, so that the size flows over the inside of the vial as a thin film. A size which flows freely, as a clear amber fluid without striations (like maple syrup) is free from gel. A size which flows freely but with striations contains gel, but of the type which dissolves within a commercially acceptable time. A size which flows rapidly in a stringy pattern contains a commercially unacceptably large amount of gel which is of the type which dissolves in too long a time. Slow flow is evidence of the presence of slow dissolving gel, and such size may appear to be free of striations and stringiness.

The comparative viscosity of the size is then determined by use of a Brookfield viscosimeter at 100 r.p.m. and 25° C.

The comparative ease with which the sizes can be diluted with cold water is determined by gently stirring with a spatula 2.5 g. of the size in each instance into 97.5 g. of water at 18° C. and recording the time required for a clear and sparkling solution to form.

Results are as follows.

| Run No.: | Monool       |               | Visc. of size <sup>1</sup>     |                            |               |               |                                   |
|----------|--------------|---------------|--------------------------------|----------------------------|---------------|---------------|-----------------------------------|
|          | Name         | Percent added | Flow mode of size <sup>2</sup> | Amount of gel <sup>3</sup> | Cp. at 25° C. | Percent decr. | Dilutability of size <sup>4</sup> |
| 1.       | Methanol     | 10            | Fast; striations               | Slight                     | 4,350         | 46.8          | 6                                 |
| 2.       | Ethanol      | 10            | do                             | do                         | 2,060         | 77.8          | 5                                 |
| 3.       | n-Propanol   | 10            | do                             | do                         | 2,670         | 71.4          | 5                                 |
| 4.       | Iso-propanol | 10            | Fast; clear                    | None                       | 2,560         | 72.5          | 3                                 |
| 5.       | n-Butanol    | 10            | Fast; striations               | Slight                     | 3,670         | 60.5          | 11                                |

<sup>1</sup> Based on solids in the size.

<sup>2</sup> Observed by reversing vials of size at 18° C. "Fast"=like maple syrup.

<sup>3</sup> See text above. "Much" indicates gel is of putty-like consistency; "slight" indicates that size is easily fluid and that only faint striations are observable during flow.

<sup>4</sup> Minutes to form clear 2.5% by weight solution, when pipetted with gentle stirring into water at 18° C.

proximately 3500 centipoises) at 15.5° C., and dissolves rapidly when stirred into ice water.

The size prepared above imparts substantially the same water-resistance to paper as the size described in Examples 1-3.

The size of Example 4 illustrates our discovery that size of extraordinary fluidity and dispersibility in cold water is achieved when the size contains substantially no free rosin acid, when substantially all of the metal cations in the size are potassium, and when the amount of monool in the size is between about 8% and 12% of the weight of size solids in the size. At 71° C. these sizes are fluid liquids even when their size solids content is as much as 70% by weight.

#### Example 5

The following illustrates the comparative effectiveness of a number of C<sub>1</sub>-C<sub>4</sub> monoools in paste rosin sizes of the present invention.

A master batch of paste rosin size is prepared by heating 600 g. (2.3 mols or equivalents) of commercial fortified rosin (tall oil rosin fortified by a content of  $\frac{2}{10}$  mol of fumaric acid), adding 246.5 g. of a 45.6% by weight solution of potassium hydroxide in water 2.0 mols) and 51.9 g. of water with stirring, and maintaining the reaction mixture at 90° C. with stirring. The water lost by evaporation is then replaced; the product is paste size weighing 898.4 g. of which 676.4 g. (75.3% is solids.

#### We claim:

1. Fluid rosin size of between about 65% and 85% solids content which is of pumpable viscosity at standard storage temperatures and which uniformly dissolves to a clear solution when one part by weight is stirred with 99 parts by weight of water at 40° C., consisting essentially of an aqueous dispersion of a rosin at least about 85% saponified with an alkali metal alkali at least about 75 mol percent of the metal cations which are potassium, and as an anti-gel agent, between about 9% and 20% (based on the weight of rosin size solids in said size) of a C<sub>1</sub>-C<sub>4</sub> saturated monool, the rosin size solids content of said size being between about 65% and 80% by weight and the weight of water in said size being greater than the weight of said monool.

2. Rosin size according to claim 1 which when of 60%-75% rosin size solids content disperses readily in water at 20° C. wherein the rosin is more than 85% neutralized, the weight of the monool is 9%-12% of the weight of rosin size solids in the size, more than 85 mol percent of the metal ions in said size are potassium ions, and the temperature of said size is below 100° F.

3. Rosin size according to claim 2 wherein the rosin is more than 95% neutralized and wherein more than 95 mol percent of the metal ions are potassium, said size being of pumpable viscosity at room temperature and being readily soluble to 1% solids in ice water.

4. Size according to claim 1 wherein the rosin is a fumarated rosin.

5. Size according to claim 1 wherein the rosin is more than 95% saponified.

6. Size according to claim 1 wherein substantially all 5 of the metal cations therein are potassium.

7. Size according to claim 1 wherein the monool is isopropyl alcohol.

8. Size according to claim 1 wherein the monool is 10 ethanol.

**References Cited****UNITED STATES PATENTS**

|           |         |                   |       |         |
|-----------|---------|-------------------|-------|---------|
| 2,262,454 | 11/1941 | Flenner           | ----- | 106—237 |
| 2,873,203 | 2/1959  | Hopkins et al.    | ----- | 106—238 |
| 3,321,325 | 5/1967  | Wisenbaker et al. | ----- | 106—239 |

JULIUS FROME, *Primary Examiner.*

T. MORRIS, *Assistant Examiner.*

U.S. Cl. X.R.

106—237; 162—180; 260—97